

# UNITED STATES PATENT OFFICE.

PORTER H. BRACE, OF PITTSBURGH, PENNSYLVANIA, ASSIGNOR TO WESTINGHOUSE ELECTRIC & MANUFACTURING COMPANY, A CORPORATION OF PENNSYLVANIA.

## METHOD OF FORMING ALLOYS.

1,355,532.

Specification of Letters Patent.

Patented Oct. 12, 1920.

No Drawing.

Application filed April 18, 1919. Serial No. 291,034.

To all whom it may concern:

Be it known that I, PORTER H. BRACE, a citizen of the United States, and a resident of Pittsburgh, in the county of Allegheny and State of Pennsylvania, have invented a new and useful Improvement in Methods of Forming Alloys, of which the following is a specification.

My invention relates to a method of forming alloys and more particularly alloys of nickel with tantalum, columbium or other metals of the tantalum group.

Heretofore, considerable difficulty has been met with in forming alloys of this character because of the marked affinity which the tantalum or its equivalent metal has for oxygen and nitrogen. On account of the readiness with which the tantalum will combine with oxygen and nitrogen and also because of the high temperatures required to melt the tantalum, it has previously been necessary to perform the entire process *in vacuo*, with the result that commercial production was almost prohibitive.

The primary object of my invention resides in providing a method of forming alloys of this character such that only a portion of the operation need be carried out *in vacuo* and such as will materially reduce the working temperatures required.

I have found that alloys of nickel and tantalum or a metal of the tantalum group may be readily formed, in any desired proportions, by reducing mixed oxids of the metals employed, to form carbids, and by subsequently melting the carbids, thus formed, *in vacuo*.

In practising my invention, I may mix suitable proportions of nickel oxid and an oxid of a metal of the tantalum group, as, for example, tantalum oxid in suitable proportions, dependent upon the relative proportions of the tantalum and nickel desired in the alloy. I may then fuse the mixed oxids, with an excess of carbon, in a furnace, the atmosphere of which is reducing, as, for example, a carbon-resistance electric furnace, to form carbids of the metals. As these carbids have relatively slight affinity for oxygen and nitrogen, this operation need not be performed *in vacuo*.

After the mixture of the metallic carbids has been formed, they may be melted *in vacuo* in the presence of tantalum oxid in sufficient quantities to remove the carbon and any gaseous impurities. This melting *in vacuo* of the mixed brittle carbids, provided by the previous step of the process, yields a silvery-white, malleable alloy of nickel and tantalum.

Although I have described my invention in connection with the production of nickel and tantalum alloys, it will be appreciated that it may be employed in the formation of all alloys to which it is adaptable and it will also be understood that any changes, which may seem desirable, may be made without departing from the spirit of my invention, as set forth in the appended claims.

I claim as my invention:

1. The method of forming metallic alloys which comprises mixing oxids of the metals to be alloyed, reducing them with an excess of carbon to form carbids, and subsequently melting the carbids *in vacuo* in the presence of an oxid of one of the metals.

2. The method of forming an alloy of nickel and a metal of the tantalum group which comprises forming a mixture of the oxids of the metals, reducing the oxids with an excess of carbon to provide carbids and melting the carbids *in vacuo* in the presence of an oxid of the metal of the tantalum group.

3. The method of forming an alloy of nickel and tantalum which comprises mixing oxids of nickel and tantalum with an excess of carbon, reducing the mixture to form carbids and melting the carbids *in vacuo* in the presence of tantalum oxid.

4. The method of forming ductile alloys of nickel and tantalum which comprises reducing the mixed oxids of the metals by means of carbon and subsequent purification of the resultant product by fusion *in vacuo* with tantalum oxid.

In testimony whereof, I have hereunto subscribed my name this 3rd day of April, 1919.

PORTR H. BRACE.